

1

2,963,420

**METHOD OF IMPROVING OLEFINIC GASOLINE BLENDING COMPONENTS**

Weldon G. Annable, Robert M. Haines, and William L. Jacobs, Crystal Lake, Ill., assignors to The Pure Oil Company, Chicago, Ill., a corporation of Ohio

No Drawing. Filed Nov. 24, 1958, Ser. No. 775,715

10 Claims. (Cl. 208—144)

This invention relates to a method of improving olefinic gasoline blending components. More particularly, it has been discovered that the sensitivity, cleanliness, and engine performance of gasoline blending components which contain more than about 40 vol. percent olefins are significantly improved by catalytic hydrogenation under specific conditions whereby the more reactive olefins are reduced to the lowest level possible without affecting the leaded research octane number of the products. The invention is directed to a specific hydrogenation treatment and to conditions found to be applicable to particular selected fractions of catalytically cracked gasolines.

Modern automotive engines have required fuels of increasingly high anti-knock quality, and the petroleum industry has responded by adopting a number of specialized processes for upgrading the octane number of gasoline blending components. One of the most widely employed present-day processes is catalytic cracking, in which paraffinic petroleum fractions are broken down into lighter olefinic and paraffinic hydrocarbons. Another widely used process is polymerization, wherein light olefinic molecules combine to form heavier olefinic molecules boiling within the gasoline boiling range. In the products of both of these types of processes, the higher octane numbers are contributed by the olefinic constituents.

While these olefin-containing gasoline blending components possess high octane ratings, they are sensitive; that is, the numerical difference between the research method octane number and the motor method octane number is high. These high sensitivities are reflected in unsatisfactory fuel performance in the more recently developed engines. It is one of the features of this invention to provide a means for reducing the sensitivities of these fuels without deleteriously affecting research-method and road-octane ratings. In essence, the motor-method octane number is raised without reducing the research-method octane rating.

When the olefin-containing, catalytically cracked, and polymeric gasolines are used in modern, compact, high-temperature engines, trouble is also experienced in the formation of deposits within the induction systems and other parts of the engines. The fuels are said to be "dirty." It is a second feature of this invention to provide a means for reducing the "dirtiness" resulting from these fuels without deleteriously affecting the research-method octane rating and road performance.

In general, the prior art has recognized the undesirability of the sensitivity of olefinic containing gasolines, and has been partially successful in overcoming it by a number of similar means. For example, the blending characteristics of olefins and paraffins are such that the olefin content of a blend containing both can be reduced to about 50%, by compositing the olefin-containing constituent with a paraffinic constituent, without markedly decreasing the research octane rating. The motor-method octane

2

rating is increased, thereby decreasing sensitivity. An analogous result can be achieved by completely saturating, by hydrogenation, a portion of the full-boiling-range material, and recombining the hydrogenated portion with the remaining olefin-containing portion in a ratio such that the total olefin content of the recombined material is only about 50% v. It is apparent that both methods consist essentially of blending olefinic and paraffinic materials. While these methods have been successful in reducing sensitivity, they have had little or no effect on the "dirtiness" caused by the final composition.

In accordance with this invention, it has been found that both the sensitivity and "dirtiness" can be markedly decreased, without deleteriously affecting research octane number or road performance, by partially hydrogenating the olefinic constituents of cracked and polymeric gasolines to reduce the olefin content to about 30-75% v., depending on the original olefin content. The maximum extent of saturation possible is also dependent on the characteristics of the particular material being treated.

By employing the instant process, reduced sensitivity is achieved as with the prior art methods described above, i.e., a balanced ratio between low sensitivity with low-octane paraffinic constituents and high sensitivity with high-octane olefinic constituents is achieved. But in addition to this, the instant process simultaneously achieves increased cleanliness, which has not been possible by prior art methods. It becomes a primary object of this invention to provide a method whereby the sensitivity and "dirtiness" of olefin-containing gasoline blending components are significantly reduced by hydrotreating the olefin-containing material at conditions such that the olefin content of the material is reduced to the greatest extent possible without deleteriously affecting research octane number.

Another object of the invention is to provide a process for improving the quality of olefinic gasoline by controlled hydrogenation using certain prescribed amounts of hydrogen whereby the desired reduction of olefinic content is obtained.

A particular feature of this invention is the finding that, contrary to the prior art, the degree or extent of hydrogenation of the olefinic constituents in an olefinic gasoline cannot be controlled by temperature regulation, pressure regulation or space velocity to accomplish the improvements sought herein, but that the degree of hydrogenation is a direct function of the amount of hydrogen present or made available for the reaction. Another feature of the invention is the discovery that this type of hydrogenation reaction must be carried out at or above a particular minimum or threshold temperature before the extent of hydrogenation becomes a function of available hydrogen, regardless of pressure, space velocity, further increases in temperature, etc., to obtain the results as will be hereinafter described.

In order to illustrate the invention, the following examples are given:

**EXAMPLE 1**

A conventional "cat. poly." gasoline was subjected to catalytic hydrogenation over a catalyst consisting of 9% molybdena on alumina (Filtrol R-3241). At a temperature of 500° F., pressure of 300 p.s.i.g., liquid space velocity of 2.5 v./hr./v., and hydrogen rate of 2000 ft.<sup>3</sup>/bbl. of hydrocarbon charge, hydrogenation did not take place to any measurable extent. On the other hand, when the temperature was raised to 625° F. while holding the other conditions constant, complete hydrogenation occurred. When space velocity was increased to 9.85 v./hr./v., at 625° F. and 300 p.s.i.g., the degree of hydrogenation was

controllable by varying the hydrogen rate. The following results were obtained:

Table I

| H <sub>2</sub> Rate (s.c.f./bbl.) | Product                    |                |              |                      |
|-----------------------------------|----------------------------|----------------|--------------|----------------------|
|                                   | Olefin Content, Percent v. | Octane Numbers |              | Sensitivity (leaded) |
|                                   |                            | MON (+3 cc.)   | RON (+3 cc.) |                      |
| (charge).....                     | 100                        | 86.0           | 101.4        | 15.4                 |
| 465.....                          | 77.8                       | 89.0           | 101.2        | 12.2                 |
| 710.....                          | 56.3                       | 90.3           | 100.4        | 10.1                 |
| 931.....                          | 37.1                       | 90.1           | 96.1         | 6.0                  |
| 949.....                          | 29.3                       | 91.0           | 95.7         | 4.7                  |
| 1,130.....                        | 15.0                       | 91.6           | 93.9         | 2.3                  |

As can be seen, 22.2% v. of the olefinic constituents was saturated at a hydrogen rate of 465 s.c.f./bbl., reducing the sensitivity of the product by 3.2 units without substantial loss in RON. The resulting fuel was cleaner and had improved performance characteristics.

## EXAMPLE 2

Light FCC gasoline, having an ASTM distillation endpoint of 160° F., and containing 49.0% v. olefinic hydrocarbons, was subjected to mild hydrotreating over the catalyst used in Example 1. Partial hydrogenation was achieved at 650° F., 300 p.s.i.g., and 10 v./hr./v. by varying the hydrogen in a lower range than was effective in treating polymer gasoline. At a temperature of 625° F., substantially no hydrogenation occurred. Experimental results were as follows:

Table II

| H <sub>2</sub> Rate (s.c.f./bbl.) | Olefin Content, Percent v. | Octane Numbers |              | Sensitivity (leaded) |  |
|-----------------------------------|----------------------------|----------------|--------------|----------------------|--|
|                                   |                            | MON (+3 cc.)   | RON (+3 cc.) |                      |  |
|                                   |                            |                |              |                      |  |
| (charge).....                     | 49.0                       | 89.1           | 100.6        | 11.5                 |  |
| 301.....                          | 34.2                       | 91.2           | 100.5        | 9.3                  |  |
| 468.....                          | 20.8                       | 94.0           | 98.7         | 4.7                  |  |
| 696.....                          | 7.4                        | 97.0           | 97.6         | 0.6                  |  |
| 890.....                          | 3.9                        | 97.6           | 97.1         | -0.5                 |  |

From these data, it is apparent that reducing the olefin content of the light FCC gasoline to about 34%, reduced sensitivity by 2.2 units without substantial loss in RON. The resulting fuel showed improved cleanliness and engine performance.

## EXAMPLE 3

The necessity for having an olefin content greater than about 40% in blending components to be treated in accordance with our invention was demonstrated by partially hydrogenating a full-boiling-range FCC gasoline over the catalyst used in the previous examples. It was found necessary to increase the reaction temperature to 700° F. to induce partial hydrogenation. Experimental results were as follows:

Table III

| H <sub>2</sub> Rate (s.c.f./bbl.) | Product                    |                |              |                      |
|-----------------------------------|----------------------------|----------------|--------------|----------------------|
|                                   | Olefin Content, Percent v. | Octane Numbers |              | Sensitivity (leaded) |
|                                   |                            | MON (+3 cc.)   | RON (+3 cc.) |                      |
| (charge).....                     | 31.6                       | 87.3           | 98.8         | 11.5                 |
| 685.....                          | 23.0                       | 88.0           | 97.6         | 9.6                  |
| 985.....                          | 13.6                       | 88.7           | 96.5         | 7.8                  |
| 976 <sup>1</sup> .....            | 1.4                        | 90.0           | 94.8         | 4.8                  |

<sup>1</sup> Space velocity reduced to 5 v./hr./v.

From these data, it is apparent that a fuel of better performance cannot be prepared by our method when the

olefin content of the material to be treated is less than about 40% v.

In order to further illustrate the invention, a series of experiments were conducted using the same catalytic polymer gasoline and hydrogenation catalyst as in Example 1, but the process conditions were varied in order to detect the influence on the percentage of olefin saturation. The following tabulation illustrates the conditions and saturation results of these experiments.

Table IV

## HYDROGENATION OF CAT. POLY. GASOLINE

| Run No.  | Temp. (° F.) | Press. (p.s.i.g.) | LVHSV             | H <sub>2</sub> Rate (s.c.f./bbl.) | Saturation (percent) |
|----------|--------------|-------------------|-------------------|-----------------------------------|----------------------|
| 241..... | 550          | 100               | 2.5               | 1,990                             | 0                    |
| 244..... | 553          | 100               | 2.56              | 1,890                             | 0                    |
| 245..... | 554          | 300               | 2.64              | 1,940                             | 3.6                  |
| 246..... | 553          | 500               | 2.47              | 1,960                             | 6.0                  |
| 247..... | 605          | 300               | 2.45              | 1,980                             | 99.3                 |
| 248..... | 600          | 500               | 2.5               | 1,920                             | 100.0                |
| 250..... | 602          | 300               | 2.53              | 940                               | 92.9                 |
| 251..... | 599          | 300               | 2.55              | 2,900                             | 99.6                 |
| 252..... | 577          | 300               | 4.99              | 1,980                             | 97.9                 |
| 253..... | 631          | 300               | 5.00              | 920                               | 88.7                 |
| 254..... | 627          | 300               | 9.91              | 470                               | 22.2                 |
| 255..... | 627          | 300               | 9.85              | 710                               | 43.7                 |
| 256..... | 629          | 300               | 9.74              | 930                               | 62.9                 |
| 257..... | 630          | 300               | 1 <sup>1</sup> 10 | 950                               | 70.7                 |
| 258..... | 634          | 300               | 1 <sup>1</sup> 10 | 1,130                             | 85.0                 |
| 266..... | 654          | 300               | 1 <sup>1</sup> 10 | 820                               | 70.3                 |

<sup>1</sup> Approximation.

The characteristics of the several charge stocks are given in Table V following.

Table V

## INSPECTION DATA ON CHARGE STOCKS

| 35 | Property                                   | Cat. Poly. | Light FCC 7D-587 | Full Range FCC 7D-445 |
|----|--------------------------------------------|------------|------------------|-----------------------|
| 40 | Gravity, ° API.....                        | 64.5       | 81.2             | 58.3                  |
|    | Reid Vapor Press., p.s.i.....              | 6.5        | 13.9             | 8.0                   |
| 45 | ASTM Distillation, ° F.:                   |            |                  |                       |
|    | IBP.....                                   | 104        | 90               | 100                   |
|    | 5%.....                                    | 185        | 99               | 113                   |
|    | 10%.....                                   | 217        | 101              | 120                   |
|    | 20%.....                                   | 241        | 103              | 131                   |
|    | 30%.....                                   | 254        | 106              | 143                   |
|    | 40%.....                                   | 265        | 110              | 162                   |
|    | 50%.....                                   | 276        | 114              | 196                   |
|    | 60%.....                                   | 286        | 119              | 238                   |
|    | 70%.....                                   | 297        | 125              | 283                   |
|    | 80%.....                                   | 309        | 134              | 322                   |
|    | 90%.....                                   | 333        | 144              | 359                   |
|    | 95%.....                                   | 372        | 150              | 382                   |
| 50 | E.P. ....                                  | 412        | 166              | 393                   |
|    | Rec. ....                                  | 98.0       | 99.0             | 98.0                  |
|    | Res. ....                                  | 1.2        | 0.6              | 1.1                   |
|    | Loss. ....                                 | 0.8        | 0.4              | 0.9                   |
|    | Refractive Index, $n^{20}/D$ .....         | 1.4120     | 1.3780           | 1.4220                |
| 55 | Vol. Percent Naphthenes and Paraffins..... | 0          | 50               | 43                    |
|    | Vol. percent Olefin.....                   | 100        | 49               | 32                    |
|    | Vol. percent Aromatics.....                | 0          | 1                | 25                    |
|    | Wt. percent Sulfur.....                    | 0.006      | 0.017            | 0.025                 |
| 60 | Research Octane—<br>+0.0 ml. TEL.....      | 97.5       | 94.0             | 93.4                  |
|    | +3.0 ml. TEL.....                          | 101.4      | 100.6            | 98.8                  |
|    | Motor Octane—<br>+0.0 ml. TEL.....         | 82.0       | 83.3             | 80.9                  |
|    | +3.0 ml. TEL.....                          | 86.0       | 89.1             | 87.3                  |
|    | Sensitivity @ 3.0 ml. TEL.....             | 15.4       | 11.5             | 11.5                  |

Referring to Table IV, runs 241 and 244 show that at the 550° F., 100 p.s.i.g., and 2.5 LVHSV level, even with an H<sub>2</sub>-rate of near 2000 s.c.f./bbl., no reaction occurred. In runs 245 and 246, the only substantial change was pressure, and at best only 6.0% saturation resulted. Runs 247 and 248 show that under these pressure, space-velocity and H<sub>2</sub>-rate conditions, an increase in temperature to 600–605° F. brought about complete saturation. The balance of the runs, that is, 250 to 266, were at or above this threshold temperature and all were at 300 p.s.i.g. pressure. A comparison of runs 247 and 248 with run 250 shows that a drop in H<sub>2</sub>-rate caused a drop in percent saturation. Comparison of runs 250 and 251 shows that an increase in H<sub>2</sub>-rate increased the percent saturation, even though it was already at a 92% level.

On the other hand, comparing runs 251 and 252 shows that increasing or even doubling the space velocity had no effect on the percent saturation, but in run 253 a reduction in H<sub>2</sub>-rate caused a reduction in percent saturation. In run 254, a further increase in space velocity and reduction in H<sub>2</sub>-rate caused a large decrease in percent saturation. In comparing runs 254 and 255 at the same temperature, pressure and space velocity, it is seen that an increase in H<sub>2</sub>-rate again doubled the percent saturation, and in run 256 a further increase in H<sub>2</sub>-rate under these same conditions caused another jump in percent saturation. Runs 257, 258 and 266 show these same effects of H<sub>2</sub> rate at the 70% saturation level. Thus it is important that the reaction be conducted at a temperature of at least about 600° F. with an H<sub>2</sub>-rate of more than 920 s.c.f./bbl. of feed, regardless of pressure and space velocity, in order to attain a saturation of from 70% to 25%, or to leave an olefin content of 30% to 75%.

In conducting the process of hydrogenation of olefinic gasoline blending components in accordance with this invention, it is only necessary to use a gasoline having 40% by volume or more of olefinic components and subject this gasoline to hydrogenation at a temperature of at least about 600° F., at elevated pressures, at a liquid volume hourly space velocity of at least about 2.5, and control the hydrogen rate within the limits of about 400 s.c.f./bbl. to 3000 s.c.f./bbl. to reduce the olefin content to the lowest level possible without affecting the leaded research octane number, that is, to reduce the olefinic content to between about 30% to 75% by volume depending on the olefin content of the original feed gasoline. Where the original olefin content is about 90-100% by volume, the maximum decrease in leaded sensitivity is attained, without deleteriously affecting the research octane number and attaining the maximum appreciation in motor octane level, at an olefin content of about 70% to 80%. In the lower range of original olefin content, between above about 40% by volume up to 60% by volume, the final olefinic content should be about 32% by volume to 36% by volume to attain maximum reduction in leaded sensitivity without loss in research octane number.

These results are readily and consistently obtainable through controlling the hydrogenation reaction by limiting the amount of hydrogen available for the reaction, i.e., by limiting the volume of hydrogen per volume of feed while maintaining a threshold temperature of at least about 600° F., regardless of pressure or space velocity. This concept is contrary to customary ways of controlling hydrogenation reactions. For example, in general the art teaches that the degree of hydrogenation can be controlled by control of any one of the usual variables. It is often stated in the art that using the same catalyst at the same temperature with the same amount of hydrogen, and at through-puts of about 1.5 to 2 v.v./hr., the pressure is maintained at lower values so as to cause partial saturation of the feed hydrocarbon. The instant experiments prove that this mode of operation is not controlling, establish that space velocities are not controlling, and that a threshold temperature must be reached before the desired partial hydrogenation can be accomplished. Furthermore, the process need not be applied to special fractions of the olefinic gasoline to attain maximum benefits with respect to leaded sensitivity and octane appreciation.

In carrying out the method of this invention, the hydrogenation may be carried out batch-wise or continuously in the presence or absence of a catalyst. However, it is preferred that a catalyst be used as long as the method is capable of saturating only the more reactive olefinic components, and for this purpose any catalyst having hydrogenation activity may be used. Suitable catalysts include oxides and sulfides of group VI and VIII metals, and more specifically oxides of cobalt or

5  
6  
molybdenum, Raney nickel, nickel sulfide, tungsten sulfide, molybdenum sulfide, and mixtures of metal sulfides or oxides, used alone or on a carrier such as alumina, clay, pumice, etc. Satisfactory results are obtained with a catalyst consisting of 9% by wt. of molybdenum on an alumina support. The feed stock to be treated is vaporized, mixed with the required amount of hydrogen and passed over a catalyst in a reaction zone heated to about 600° F. or higher if necessary. The conditions of pressure and space velocity are regulated to values sufficient to allow the reaction to begin and the degree of hydrogenation is controlled by regulation of the amount of hydrogen available for the reaction.

Feed stock for the process of this invention includes those blending components, boiling within the gasoline boiling range, i.e., about 100° F. to 400° F., which contain more than 40% by volume of olefins. Example feed stocks are polymer gasolines, the low-boiling portions of fluid-catalytic-cracked gasolines, and various fractions of these types of materials. In general, where the fraction being treated has an olefin content of 90%-100% by volume, the amount of hydrogen used is adjusted to reduce the olefin content about 18-20%. In using an FCC gasoline where the original olefin content is 45 to 52% by volume, it is only necessary to adjust the amount of hydrogen so as to reduce the olefin content by an amount equal to about 10% to 20%.

What is claimed is:

1. The process of decreasing the sensitivity of olefinic gasoline blending stocks containing at least about 40 percent by volume of olefins which comprises subjecting said blending stocks to hydrogenation at a temperature of at least about 600° F., a pressure of at least about 100 p.s.i.g., a liquid volume hourly space velocity of at least about 2.5 and controlling the amount of hydrogen during the reaction to between about 400 to 2000 s.c.f./bbl. as the reaction proceeds to attain the greatest increase in motor octane research number with the least decrease in research octane number.

2. The process of decreasing the sensitivity of a catalytic polymer gasoline containing at least about 40 percent by volume of olefins which comprises subjecting said catalytic polymer gasoline to hydrogenation at a temperature of at least about 600° F., a pressure of at least about 100 p.s.i.g., a liquid volume hourly space velocity of at least about 2.5 and controlling the amount of hydrogen during the reaction to between about 400 to 2000 s.c.f./bbl. as the reaction proceeds to attain the greatest increase in motor octane research number with the least decrease in research octane number.

3. The process in accordance with claim 1 in which the feed blending stock is a catalytic polymer gasoline having an olefin content of about 100% by volume and about 18% to 20% by volume of said olefins are hydrogenated during said reaction.

4. The process in accordance with claim 3 in which said reaction is conducted at a temperature of about 625° F. at a pressure of about 300 p.s.i.g. using a liquid volume hourly space velocity of about 2.5 with the amount of hydrogen regulated at 465 to 710 s.c.f./bbl.

5. The process in accordance with claim 1 in which the blending stock is an FCC gasoline having an ASTM end-point of 160° F. and contains about 49.0 volume percent of olefins and about 10% to 20% by volume of said olefins are hydrogenated during said reaction.

6. The process in accordance with claim 5 in which said reaction is conducted at a temperature of about 650° F. at 300 p.s.i.g. with a liquid volume hourly space velocity of about 10 and using about 300 s.c.f./bbl. of hydrogen.

7. The method of treating an olefinic gasoline to decrease the sensitivity and tendency to form induction system deposits which comprises subjecting an olefinic gasoline containing about 100% by volume of olefinic hydrocarbons, and characterized by having an MON of about

86.0, a RON of about 101.4, and a leaded sensitivity of about 15.4, to catalytic hydrogenation in the presence of a molybdena-alumina catalyst at a temperature of at least about 600° F. using pressures of about 300 p.s.i.g. under a space velocity of about 9.85 v./hr./v. and controlling the hydrogen rate to about 465 s.c.f./bbl., continuing said reaction until the olefin content of the product is about 77.8 volume percent and recovering a product having a decreased leaded sensitivity, an increased MON and substantially the same RON.

8. The method in accordance with claim 7 in which the olefinic gasoline is a catalytically polymerized gasoline.

9. The method in accordance with claim 7 in which the olefinic gasoline has an olefinic content of at least 15 10 40% by volume.

10. The method in accordance with claim 7 in which the temperature is maintained at about 625° F. throughout the reaction.

References Cited in the file of this patent

UNITED STATES PATENTS

|           |                   |                |
|-----------|-------------------|----------------|
| 2,289,716 | Marschner         | July 14, 1942  |
| 2,434,577 | Miller            | Jan. 13, 1948  |
| 2,458,980 | Cole              | Jan. 11, 1949  |
| 2,694,671 | Baumgarten et al. | Nov. 16, 1954  |
| 2,717,861 | Baumgarten et al. | Sept. 13, 1955 |
| 2,810,004 | Morbeck et al.    | Oct. 15, 1957  |
| 2,861,946 | Sage et al.       | Nov. 25, 1958  |